

W. D. COOLIDGE.  
REFRACTORY CONDUCTOR.

APPLICATION FILED AUG. 1, 1906. RENEWED DEC. 8, 1910.

1,026,429.

Patented May 14, 1912.



Witnesses:

George H. Pilden  
Helen Oxford

Inventor:  
William D. Coolidge,  
by *Albert B. Davis*  
Att'y.

# UNITED STATES PATENT OFFICE.

WILLIAM D. COOLIDGE, OF SCHENECTADY, NEW YORK, ASSIGNOR TO GENERAL ELECTRIC COMPANY, A CORPORATION OF NEW YORK.

## REFRACTORY CONDUCTOR.

1,026,429.

Specification of Letters Patent.

Patented May 14, 1912.

Application filed August 1, 1906, Serial No. 328,726. Renewed December 8, 1910. Serial No. 596,373.

To all whom it may concern:

Be it known that I, WILLIAM D. COOLIDGE, a citizen of the United States, residing at Schenectady, county of Schenectady, State 5 of New York, have invented certain new and useful Improvements in Refractory Conductors, of which the following is a specification.

This invention relates to the production 10 of refractory electrical conductors suitable for use in incandescent lamps, electric furnaces, and other apparatus.

It comprises a process whereby refractory material, even though non-ductile, may be 15 shaped into wires, plates, rods, or other forms, and then consolidated into a coherent conductor capable of converting electrical energy into light at enormously high temperatures.

20 According to my invention, a refractory element, alloy, compound or mixture is impregnated with a ductile metal or alloy, and the product so obtained is sintered together and consolidated by the passage of current 25 therethrough, either before or after mechanical manipulations of the material, such as rolling, drawing, squirting, etc.

My process is applicable to a great variety 30 of refractory metals and materials, such for instance, as tungsten, molybdenum, boron, zirconium, titanium, or compounds or alloys of any of these, or of other material of the same general refractory nature. The less refractory metals or alloys with 35 which these refractory materials are impregnated, may be such metals as copper, cadmium, gold, silver, mercury, bismuth, tin, and various other of the well known metals having vaporizing points approximating those of the metals above named; or 40 I may use amalgams or other alloys of these metals, such for instance as cadmium, amalgam, bismuth-cadmium alloy or bismuth-cadmium-mercury alloy, etc. In general, 45 the less refractory metals are introduced into the pores of the refractory material and serve to give the body ductility and strength, and in some cases to increase its electrical conductivity. The ductile or low melting 50 metal is retained in this position until the body has been worked or formed into the desired shape and it is then driven out by heat treatment to leave behind a refractory wire or rod.

55 My process may be carried out with the

aid of divers forms of apparatus, but I have shown in the drawings forming a part of this specification, one means for effecting the desired result, and in the following description I have indicated other means for carrying out the general idea of my invention.

In the drawings, Figure 1 is an elevation of one type of electric furnace in which the impregnating process may be effected; Fig. 65 2 is a sectional elevation of a crucible and its charge, suitable for use in an electric furnace of somewhat different construction.

In Fig. 1, a hermetically sealed chamber 1 of glass or other suitable material, is provided at its top with an opening 2 through which passes a metal rod or plunger 3, carrying at its lower end a plurality of clips 4, which engage with one end of a block or rod of refractory material to be treated. This 75 block or rod consists of pure tungsten powder pressed into shape under heavy pressure, though it is to be understood that other materials than tungsten may be treated in a similar manner, or that the rod may be made 80 by other known methods. The rod or plunger 3 passes into the chamber through a rubber pressure tubing 6 and makes an air tight joint therewith so that it may be raised or lowered without materially affecting 85 the state of the vacuum within the chamber. The rod also serves to establish an electrical connection to the tungsten block for purposes hereinafter set forth. The tube or chamber 1 is permanently connected 90 to a suitable vacuum pump so that the gases or vapors given off during the treatment may readily be removed. At the bottom of the chamber or envelop 1 is placed a quantity of the ductile metal, amalgam or alloy 95 with which the tungsten is to be impregnated. If this metallic material is not liquid at ordinary temperatures, I may heat the lower end of the tube with a flame or with a suitable liquid bath 8. This bath 100 may consist of molten type metal, lead, or even of higher melting elements or compounds, provided the temperature does not exceed that at which the glass or other envelop will successfully operate. Electrical 105 connection may be established to the metal 7 through suitable lead wires 9 passing through the envelop. In utilizing this apparatus, I first exhaust the air from the chamber and then lower the plunger with 110

its supported rod or block of tungsten until the latter makes contact with the liquid metal in the lower part of the envelop. The plunger is then lifted and an arc established between the tungsten rod and the vaporizable metal at the bottom of the tube. Preferably this metal acts as the cathode for a direct current arc. The tungsten rod, when subjected as anode to the heating action of the metallic arc, gives off considerable quantities of occluded air and other gases, and these are taken out through the pump, so that after some minutes of operation the tungsten rod is in a clean and porous condition and well adapted to receive metal within its pores. When this condition is reached I suddenly lower the tungsten rod into the liquid metal and permit the ductile metal to percolate through the tungsten and completely fill up all the minute spaces in the stick. It is not necessary that all the tungsten rod should be submerged in the fused metal as I find that the ductile metal is drawn up by capillary or similar forces into all parts of the stick which have been highly heated. I next withdraw the impregnated stick from the liquid, and after cooling, I remove it from the tube and break away the extreme end which was in contact with the spring clips 4, for fear that this end might perchance have been contaminated by contact with the clips. The resulting stick is smooth and strong, has a fine even fracture and may readily be polished. I find that the quantity of ductile metal taken up by the refractory pressed stick depends on the degree of subdivision of the refractory powder and also on the extent to which it has been compressed. The color of the resulting stick is also dependent on the ductile metal used; in general the impregnated material resembles the ductile material. Tungsten impregnated with silver or cadmium is white, while tungsten or the other refractory metals become yellow or salmon colored when impregnated with copper.

In impregnating with copper and other ductile metals which fuse at temperatures somewhat higher than would be conveniently obtained in the apparatus shown in Fig. 1, I utilize the crucible shown in Fig. 2, together with a vacuum furnace of the type shown in United States Patent to Arsem No. 785,535, March 21, 1905. The crucible 10, shown in Fig. 2, may consist of graphite, alumina or other material which is inert with respect to the materials under treatment, at the temperature of treatment. The ductile or fusible metal 11 is placed in the crucible, together with the pressed or molded stick of refractory material. The crucible is then introduced in the vacuum furnace, the air exhausted, and the temperature raised to the point at which gases are lib-

erated from the stick under treatment. I prefer, however, not to raise the temperature of treatment high enough to liquefy the ductile metal until after all the gases have been pumped from the refractory stick. 70 When, however, the material becomes free from occluded gases and volatile matter, I raise the temperature to liquefy the fusible metal 11, whereupon the refractory stick soaks up relatively large quantities thereof. 75 Even with sticks several inches long the liquefied metal diffuses to the extreme upper end of the stick. I next allow the crucible to cool and when it can safely be removed from the furnace I break away the treated 80 stick from the unused ductile metal and then have a product similar to that obtained by the apparatus shown in Fig. 1.

The impregnated sticks above described may be subjected, without further treatment, to the sintering or consolidating action of a high current. To do this, I provide them with suitable terminals, mount them in a vacuum or an inert atmosphere, and pass sufficient current through the sticks 85 to vaporize the less refractory metal or alloy, and leave behind a coherent sintered mass of refractory material. Whatever the principle may be which underlies this phenomenon, I find that if the current is properly applied, the resultant stick is much stronger and better suited for use as glowers than the original stick of pressed or untreated material. My process is not, however, limited to the production of refractory 90 glow bodies of relatively large cross-section, as I find that the impregnated sticks may be rolled, drawn, or extruded much like pure metals of fair ductility, and that by careful handling I can convert the sticks into plates 95 or foil or into wires and strips of substantially the size now used in incandescent lamps. All this may be done, even though the original refractory stick is pressed up from a non-coherent and finely divided powder. 100 After obtaining wires of the desired size and shape, I draw out the ductile metal by current passed therethrough, and I sinter the refractory particles together so strongly 105 that the resulting filament appears to be a compact uniform wire of homogeneous structure. If I work with material as refractory as tungsten, titanium or other metals above enumerated, the refractory filaments produced may be operated in an incandescent lamp at an exceedingly high efficiency. 115

The rolling, drawing, or extruding operations above mentioned may under certain circumstances be facilitated by heating the 120 material under treatment, and also by heating the rolls or dies through which it passes. In fact, when pressing or squirting a stick impregnated with such materials as copper, cadmium, amalgam, etc., I consider that the 125

danger of fracturing the die may be greatly lessened by subjecting the stick to considerable heat, though I am careful not to apply enough heat to break up the bond between the ductile metal or alloy and refractory particles, or in any way to interfere with the production of a smooth, strong and uniform wire or thread of squirted material.

I have above described the impregnation of a compressed body of refractory powder by heat treatment in a vacuum followed by contact with a bath of bismuth-cadmium alloy, and have presented claims on the complete process as described. In another application Serial No. 377,781, filed by me June 7, 1907, I have presented claims of a somewhat general nature on the production of a mixture of a refractory material with bismuth-cadmium amalgam and on the production of lamp filaments therefrom, together with suitable claims on the product.

What I claim as new and desire to secure by Letters Patent of the United States is,—

1. The process which consists in shaping a body from refractory material, impregnating said body with a metallic material having a relatively low vaporizing temperature, and subsequently heating said product by current passed therethrough to vaporize said metallic material and consolidate said body.

2. The process which consists in compressing a refractory powder into a rigid body, impregnating said body with ductile metal, and subsequently passing current through said body to vaporize said ductile metal and consolidate said body.

3. The process which consists in compressing a refractory material into a predetermined shape, heating said material in a vacuum to remove gases therefrom, impregnating with a ductile metallic material, and subsequently driving out said ductile material by current passed through said body.

4. The process which consists in shaping a rigid body from refractory powder, heating said body in a vacuum to remove gases therefrom, immersing a portion of said body in a fused metallic material to impregnate said body with said material, shaping the resultant product into conductors, and subsequently heating said conductors to drive the easily fusible components therefrom.

5. The process which consists in impregnating a stick of refractory material with a less refractory metallic material, shaping the product so formed into conductors, and

subsequently treating to remove all components except said more refractory material.

6. The sub-process which consists in compressing refractory material into a stick, impregnating said stick with a ductile metallic material, and squirting the product so obtained to produce wires.

7. The process which consists in compressing refractory material into a stick, impregnating said stick with a ductile metallic material, squirting the product so obtained to produce wires, and heating said wires to remove all easily vaporizable components therefrom.

8. The process which consists in compressing a refractory powder into a rigid body, impregnating said body with a ductile metal, and subsequently heating said body to vaporize said ductile metal and consolidate said body.

9. The process which consists in compressing a refractory powder into a predetermined shape, heating said material in a vacuum to remove gases therefrom, then bringing said material into contact with a fusible metallic material to impregnate it therewith, and subsequently driving out said fusible material.

10. The process which consists in compressing refractory material into a stick, impregnating said stick with a ductile amalgam, squirting the product so obtained to produce wires, and heating said wires to remove all easily vaporizable components therefrom.

11. The process which consists in compressing a refractory powder into a rigid body, impregnating said body with a cadmium-bismuth amalgam, and subsequently heating said body to vaporize the components of said amalgam and consolidate the residue.

12. The process which consists in compressing a refractory powder into a predetermined shape, heating said material in a vacuum to remove gases therefrom, impregnating said material with a ductile amalgam, shaping the product so formed to produce wires, and subsequently heating to drive out the components of said amalgam.

In witness whereof, I have hereunto set my hand this 30th day of July, 1906.

WILLIAM D. COOLIDGE.

Witnesses:

BENJAMIN B. HULL,  
GRACE M. HANIGAN.